

C. L. COOK & J. R. PRICE.

PROCESS FOR THE SEPARATION OF ASPHALTIC COMPOUNDS FROM GANGUE.

APPLICATION FILED FEB. 17, 1914.

1,190,633.

Patented July 11, 1916.



WITNESSES:

J. A. Timney  
A. H. Kephart.

INVENTORS  
CARL L. COOK  
JOHN R. PRICE

BY

Carlos P. Griffin  
ATTORNEY.

# UNITED STATES PATENT OFFICE.

CARL L. COOK, OF SAN FRANCISCO, AND JOHN R. PRICE, OF OAKLAND, CALIFORNIA.

## PROCESS FOR THE SEPARATION OF ASPHALTIC COMPOUNDS FROM GANGUE.

1,190,633.

Specification of Letters Patent.

Patented July 11, 1916.

Application filed February 17, 1914. Serial No. 819,212.

*To all whom it may concern:*

Be it known that we, CARL L. COOK and JOHN R. PRICE, citizens of the United States, residing at San Francisco and Oakland, respectively, in the counties of San Francisco and Alameda, State of California, have invented a new and useful Process for the Separation of Asphaltic Compounds from Gangue, of which the following is a specification in such full and clear terms as will enable those skilled in the art to construct and use the same.

This invention relates to a process for the separation of asphaltic compounds from sand rock or the gangue in which such compounds are found.

It will be understood by those skilled in the art that large quantities of bitumen bearing rock or sand stone are found in nature in which the asphaltic product is too low in percentage to make the material of great value. This asphaltic compound has been heretofore extracted by various methods such as heating, boiling, or dissolving with, however, a very low percentage of extraction, and since the natural rock frequently runs as low as 14% of the asphaltic compound an extraction of only six or seven per cent. means that such an enormous quantity of the raw material must be handled as to make such a process for the recovery of the compound commercially impossible.

With this invention it is possible to obtain a high percentage extraction even when treating asphaltic rocks or sand stones containing as low as 10% asphaltum.

In the drawing in which the same numeral of reference is applied to the same portion throughout, there is illustrated a diagrammatic view partly in section of an apparatus for carrying out the process.

The numeral 1 represents the base of a boiler which has a suitable fire box fed through the door 2. The boiler is provided with a sloping bottom 3 and with the cylindrical boiler 4 around which is a heating jacket 5, the flame from the fire box impinging upon the sloping bottom 3 and passing through holes 6 and 7. At the top 50 of the heating jacket 5 and on the opposite side thereof from the hole 7 there is a smoke stack 8. At the lower portion of the sloping bottom 3 there is a discharge pipe 9 controlled by means of a quick acting valve 10, with which is connected the pipe 11. The valve stem 12 and valve connected therewith are operated by means of the handle 13 pivoted to the arm 14. In the upper portion of the boiler there is a discharge pipe 15 controlled by means of the valve 16 similar to the valve 10, this valve being operated by means of the handle 17 pivoted on the arm 18. The boiler is provided with a steam gage 19 connected therewith by means of the pipe 20. The top of the boiler is flanged outwardly as indicated at 21 and carries a plurality of bolts 22, on which bolts are the nuts 23, said bolts being hingedly connected to the flange 21 so that it is easy to disconnect them from the cover 24.

The cover 24 is hinged to the top of the boiler at 25 and when raised off the top of the boiler leans against the rest 26. When it is desired to charge the boiler the cover 24 is raised and material placed upon the platform 27 is charged into the boiler until the proper amount has been placed therein whereupon the heating is commenced.

Water is supplied to the boiler by means of the pipe 30 controlled by the valve 31. Within the boiler there is a flanged ring 32 upon which is placed a heavy wire screen 33 to prevent the materials thrown into the boiler from packing on the bottom 3 and being burned in the process of heating.

The operation of the process is as follows: The material which consists of lumps of the asphalt bearing gangue is charged into the boiler, which is partially filled with water, preferably previously raised to the boiling point. The specific gravity of the cold gangue is greater than that of the hot water and the gangue sinks through the water to the screen 33. After the charge has been introduced, the cover is secured in place, sealing the boiler, and the continued application of heat produces a temperature within the closed vessel which is in excess of 212° Fahrenheit and the temperature is increased until a pressure of from 40 to 75 pounds per square inch is produced, that is a temperature of from approximately 268° Fahrenheit to 308° Fahrenheit. As the asphalt becomes heated to 212° Fahrenheit or thereabout, its specific gravity becomes less than that of the water and it rises to the surface of the water and due to the increase in temperature it becomes somewhat plastic. This asphalt rafts to the surface with it a large amount of sand which is held by the asphalt. When it reaches the surface the asphalt is in the

form of a foamy mass, carrying in suspension a large amount of sand which is not liberated. The continued application of heat thereto however, causes the asphalt to 5 coalesce, forming substantially a perfect liquid at the temperatures which obtain and in this condition, the asphalt no longer forms a support for the sand, which settles through the water, leaving a substantially pure asphalt liquid floating on the surface.

When the asphalt has been heated for a sufficient time to cause it to coalesce or liquefy the valve 16 may be opened whereupon the asphaltic compounds will be blown 15 off. When all of the asphaltic compounds have been blown off the valve 10 may be opened and the residues which are sandy in nature may be washed out by opening the valve 31 and running a suitable supply of 20 water into the boiler. It will be observed that while heretofore it has been common to separate this material by boiling that any process of boiling involves the loss of a great amount of latent heat in the loss of the steam 25 in the boiling process, but with the present process very little heat is lost because the only steam lost is that which is lost from the mass of material after it has been discharged from the boiler, with no accompanying ebullition taking place at any time. It is also to be noted that with this process the asphaltic compounds come off comparatively pure for the reason that no ebullition takes place. It will be noted that with the 30 higher percentages of asphaltic compound present a lower pressure may be used to effect the separation than with low percentage asphaltic gangues.

Where heavy asphaltic compounds are 40 sought to be separated from the material bearing them it is necessary to add a quantity of salt (sodium chlorid) to the solution to increase its specific gravity, thereby causing the asphaltic compounds to rise to the 45 surface thereof more easily than they would in pure water.

Experiments made on asphaltic gangues show that by the process herein disclosed 50 asphaltic compounds will sink when cold and will expand sufficiently when heated to float, such action having been observed in separators used, such as are described in the diagrammatic drawing above referred to,

but it has been ascertained that to cause the material to become sufficiently light to separate properly that a pressure of from 40 to 55 80 pounds per square inch is requisite.

Having thus described our invention what we claim as new and desire to secure by Letters Patent of the United States, is as follows, modifications within the scope of the claims being expressly reserved:

1. The process of separating asphaltic compounds from gangue carrying the same, which consists in heating the gangue in 65 water to a sufficient temperature to cause the compounds to partially free themselves from the gangue and to rise through the water and continuing the heating of the floating compounds to a temperature above 212° 70 Fahrenheit whereby the compounds will coalesce and release gangue carried thereby and then separating the asphaltic compounds from the water.

2. The process of separating asphaltic 75 compounds from gangue carrying the same, which consists in heating the gangue in water to a temperature above 250° Fahrenheit whereby the asphaltic compounds are first caused to partially separate from the 80 gangue and float to the surface of the water and there to liquefy and release carried gangue which precipitates through the water and then removing the liquefied compounds from the surface of the water.

3. The process of separating asphaltic compounds from gangue carrying the same which consists in heating the gangue in water to a temperature sufficiently high to cause the compounds to partially separate 90 from the gangue and float to the surface of the water and then heating the separated compounds in water to a higher temperature whereby the compounds will coalesce and release the gangue carried thereby which precipitates through the water.

In testimony whereof we have hereunto set our hands this 11th day of February, A. D. 1914, in the presence of the two subscribed witnesses.

CARL L. COOK.  
JOHN R. PRICE.

Witnesses:

C. P. GRIFFIN,  
L. H. ANDERSON.